

Patented July 5, 1927.

1,635,025

# UNITED STATES PATENT OFFICE.

GUY M. BALL, OF DAYTON, OHIO.

## QUENCHING FLUID.

No Drawing. Application filed July 25, 1924, Serial No. 728,185. Renewed December 9, 1926.

This invention relates to a quenching fluid to be used in hardening ferrous or cuprous metals.

The primary object of this invention is 5 the provision of a quenching fluid for use in hardening metals of the above type, which has the nature of being able to very rapidly cool the metal after it has been plunged into the solution, and of cooling the metal so 10 that it will not warp or buckle.

I have found that a quenching fluid consisting of two pounds sodium chloride, one-quarter pound potassium cyanide, one pound borax, to one gallon of water gives 15 a fluid having superior properties as a quenching fluid for the hardening or tempering of wrought steel, cold rolled steel, wrought iron, and brasses and bronzes. In place of sodium chloride, the potassium salt 20 may be used. Sodium cyanide may also be used in place of the potassium cyanide, as the salt of these two metals, sodium and potassium, have similar qualities. The solution is also applicable for the treatment 25 of any other metals, the properties of which are improved by rapidly cooling in a quenching liquid. The solution is not applicable however to metals such as zinc or alloys of the same, which will be rapidly corroded and dissolved, to a large extent, when they come in contact in a heated condition with the fluid.

The solution according to the formula given in the preceding paragraph, when 35 first made, gives off a gas which has been found to be harmless to the user, but after a few hours the solution becomes stabilized, and after that time, when a heated piece of metal is plunged into it, no more dissipation of gas takes place.

The proportions as above mentioned produces a substantially saturated solution of the salts which will be of an alkaline nature, due to the presence of the borax. The 45 chemical term for the borax is either sodium borate or sodium pyroborate. It is not necessary to exactly follow the proportions as given, however, it is desirable to have sufficient amounts of the various ingredients so 50 as to form practically saturated or even a super-saturated solution, in order to obtain the best results. The amount of salt present exceeds the combined weight of the potassium cyanide and the borax as will be noted.

55 It has been found by actual test that low carbon steels, which are ordinarily diffi-

cultly tempered, are greatly hardened and tempered by being first heated to a dark cherry red color and then plunged into the solution as above outlined. A bronze specimen has been found to cool after being immersed for one second in my quenching fluid, so that in that length of time it is at a lower temperature than a similar specimen under similar conditions which is plunged into a 60 brine solution and held there for five or six seconds.

A solution prepared in accordance with my invention has qualities which equal and in some cases exceed that of oil as a quenching fluid as regards warping and buckling, together with the added advantage of very rapid cooling. The heat transfer from the heated specimen to the quenching fluid takes 70 place with my improved solution so evenly 75 and rapidly that there is very little tendency for the specimen to buckle even though it is of very thin material. The rapidity with which the heat dissipation takes place, permits results to be obtained so that the physical properties of the metal, after being so quenched, greatly exceed those which may be obtained by the use of other known formulas.

When the heated specimen is plunged into the quenching solution, the reaction at first is quite violent due to the boiling of the liquid immediately surrounding the specimen, but this reaction and turbulence in some manner appears to aid in the rapid 85 transfer of heat. With a saturated solution as before mentioned, there appears to be no formation of steam bubbles which have been thought to cause the buckling effect of brine 90 solutions. Where a specimen is plunged 95 into a brine solution it is evident that some portions of the specimen immediately after being plunged are contacting with a body of steam, while other portions are contacting with the liquid itself, and an uneven cooling 100 will take place, which will cause a warping or buckling effect. It is a comparative freedom from this effect which makes the quenching solution of my invention particularly desirable.

I claim:

1. A quenching solution for hardening metals, consisting of alkaline saturated water solution of salt, potassium cyanide, and borax.
2. A quenching solution for hardening metals, consisting of a concentrated water so-

lution of salt, potassium cyanide, and borax, the weight of salt exceeding the combined weight of the potassium cyanide and borax.

3. A quenching solution for hardening steel, iron, bronze, and brass, consisting of a concentrated solution of eight parts salt, one part potassium cyanide, four parts borax, and the remainder water.

4. A quenching solution for hardening ferrous metals, consisting of the following

ingredients in the approximate ratio named: sodium chloride, 2 lbs.; potassium cyanide,  $\frac{1}{4}$  lb.; borax, 1 lb.; water, 1 gal.

5. A quenching solution for hardening ferrous or cuprous metals comprising sodium chloride 2 pounds, potassium cyanide  $\frac{1}{4}$  pound, borax 1 pound, and water 1 gallon.

In testimony whereof I affix my signature.

GUY M. BALL.